

## UNITED STATES PATENT OFFICE

2,030,336

## PHOTOGRAPHIC DEVELOPER

Heinrich Ulrich and Karl Saurwein, Ludwigshafen-on-the-Rhein, Germany, assignors to Agfa Ansco Corporation, Binghamton, N. Y., a corporation of New York

No Drawing. Application December 22, 1933,  
Serial No. 703,672. In Germany December 24,  
1932

## 7 Claims. (Cl. 95—88)

This invention relates to a photographic developer and more particularly to such a developer in which the usual alkali or the usual preservative or both have been replaced by compounds hitherto not known for this purpose.

One of its objects is to provide a developer in which the usual alkali and the preservative are replaced by a compound uniting both functions. A further object is to replace the usual alkali compounds by compounds of which the alkalinity can be adjusted in a degree not hitherto known.

For certain purposes of photographic development it is desirable to have only a weakly alkaline developer in order to avoid drawbacks involved with the use of stronger alkaline developers.

According to this invention it has been found that the salts of hydroxyalkylamines with weak acids are excellently suited to replace for many purposes the alkali hitherto used in developers. The use of the salt of a weak acid of a hydroxyalkylamine involves the advantage that the alkalinity of the developer can be adjusted to any requirement. As hydroxyalkylamines which are suitable, there is mentioned, for instance, mono-, di- or triethanolamine, propanolamine, butanolamine, oleylethanolamine, furthermore cyclohexylethanolamine, hydroxyethylmorpholine, hydroxyethylpiperidine, hydroxyethylethylene-

30 diamine, ethyldiethanolamine or the like, further the ethers or hydroxyethers obtainable from hydroxyalkylamines by etherification with alcohols or by reaction with ethylene oxide or the like. The substitution products of the amines

35 enumerated likewise may be used. All ammonia derivatives are suitable which contain in their molecule one or several alkyl radicals with one or several hydroxy groups, and, if required, contain still further aliphatic, cycloaliphatic or mono-

40 nuclear aromatic radicals. Suitable weak acids are, for instance, carbonic acid and sulfurous acid.

The salts of hydroxyalkylamines with sulfurous acid present furthermore the advantage that they are capable to replace the preservative of 45 the usual developers. Therefore, it is possible to produce photographic developers which contain besides the developing agent the sulfite of an hydroxyalkylamine which replaces both, the usual alkali and the preservative.

50 The salts of the hydroxyalkylamines with the weak acids are easily obtainable by reacting with the compounds on each other. If the acid is gaseous, for instance, in the case of sulfuric acid, the hydroxyalkylamine is saturated with 55 the gas if the amine is liquid.

The compounds enumerated above may, for instance, be added to the developing baths customary in the photographic industry, for instance, solutions of aminophenols, hydroquinone, hydroxyphenylglycine and the like. They may also be applied in combination with other substances suitable for the development of photographic plates, films and the like, for instance with sodium bisulfite, acetone bisulfite and the like.

The following examples serve to illustrate the 10 invention:

## Example 1

|                                  |         |
|----------------------------------|---------|
| Monomethylparaminophenol sulfate | 2 grams |
| Triethanolamine                  | 5 cc.   |
| Triethanolamine sulfite          | 3 cc.   |
| Water to                         | 100 cc. |

For use this solution is diluted by 20 parts of water on one part of concentrated developer.

## Example 2

|                                  |          |
|----------------------------------|----------|
| Monomethylparaminophenol sulfate | 3 grams  |
| Triethanolamine sulfite          | 6 cc.    |
| Potassium bromide                | 0,2 gram |
| Water to                         | 500 cc.  |

## Example 3

|                                  |          |
|----------------------------------|----------|
| Water                            | 500 cc.  |
| Monomethylparaminophenol sulfate | 1,5 gram |
| Triethanolamine                  | 8 cc.    |
| Butanolamine sulfite             | 10 cc.   |
| Potassium bromide                | 1 gram   |

## Example 4

|                                  |          |
|----------------------------------|----------|
| Water                            | 500 cc.  |
| Monomethylparaminophenol sulfate | 0,3 gram |
| Hydroquinone                     | 0,4 gram |
| Sodium carbonate sicc            | 4 grams  |
| Ethanolcyclohexylamine sulfite   | 5 grams  |
| Potassium bromide                | 2 grams  |

Our invention is not limited to the foregoing examples. Other weak acid salts of other hydroxyalkylamines may be used and we contemplate as included within our invention all such modifications and equivalents as fall within the scope of the appended claims.

The term "hydroxyalkylamine" in the specification and the claims is intended to include amines containing at least one alkylhydroxy radical linked to the nitrogen atom of the amine.

What we claim is:

1. A photographic developer comprising a developing agent and a weak acid salt of a hydroxyalkylamine.

2. A photographic developer comprising a developing agent and a weak acid salt of a hydroxy-alkylamine selected from the group consisting of carbonates and sulfites.
5. 3. A photographic developer comprising a developing agent and the sulfite of a hydroxyalkyl-amine.
4. A photographic developer comprising a developing agent and a weak acid salt of a hydroxyalkyl-amine selected from the group con-10 sisting of monoethanol-amine, diethanol-amine, triethanol-amine, propanol-amine, butanol-amine, oleylethanol-amine, cyclohexylethanol-amine, hydroxyethyl-morpholine, hydroxyethyl-
- piperidine, hydroxyethylethylene-diamine, and ethyldiethanol-amine.
5. A developer comprising monomethylpara-aminophenol sulfate, triethanolamine, triethanol-amine sulfite and water.
6. A developer comprising monomethylpara-aminophenol sulfate, triethanol amine sulfite, potassium bromide and water.
7. A developer comprising monomethylpara-aminophenol sulfate, hydroquinone, sodium car-10 bonate sicc., ethanol cyclohexylamine sulfite, potassium bromide and water.

HEINRICH ULRICH.  
KARL SAURWEIN.